

Dec. 20, 1927.

1,653,124

G. A. RICHTER

## INTERRELATED PULP REFINING AND VISCOSE PROCESS

Filed Oct. 29, 1925



Inventor:

Geo. A. Richter.  
by George Braun Leinbigs May  
Atty.

Patented Dec. 20, 1927.

1,653,124

# UNITED STATES PATENT OFFICE.

GEORGE A. RICHTER, OF BERLIN, NEW HAMPSHIRE, ASSIGNOR TO BROWN COMPANY,  
OF BERLIN, NEW HAMPSHIRE, A CORPORATION OF MAINE.

## INTERRELATED PULP-REFINING AND VISCOSE PROCESS.

Application filed October 29, 1925. Serial No. 65,635.

This invention has relation to the production of viscose from cellulosic fibrous material. More particularly, it concerns itself with the production of viscose from high alpha cellulose fiber: that is, a pulp containing a high percentage of alpha or resistant cellulose.

The usual process employed in the preparation of viscose from cellulose pulp consists in subjecting air-dry pulp in sheet form (e. g., sulphite pulp) to a bath of caustic soda solution approximating 18% in concentration of caustic soda. After the sheets have been thoroughly impregnated or saturated with the caustic soda solution, they are removed from the bath and subjected to pressure in a manner to express or remove the excess caustic soda solution contained therein but to allow sufficient caustic soda to remain behind for effecting the conversion of the cellulose fiber into the soda cellulose, so called. The pressed pulp sheets with the caustic soda solution contained therein, are allowed to stand or age for two days or so, during which time a reaction takes place between the caustic soda and cellulose. There is some question regarding the precise reaction consummated between the reacting components, but it is generally assumed that the cellulose forms an addition product with the caustic soda.

The soda cellulose or addition product thus produced is then treated, preferably while agitated with the amount of carbon bisulphide necessary to form cellulose xanthate or viscose. Enough additional caustic soda and water are added during or after the completion of the reaction to permit the solution of cellulose xanthate formed by the reaction in the alkaline liquor. The resulting colloidal product may be a yellow, orange, red or greenish syrup or jell, depending upon the impurities contained in the ingredients and the physical conditions attending the reactions.

The colloidal syrup or jell thus prepared is allowed to stand or ripen to the proper degree. The ripening step requires two or three days, during which time certain spontaneous chemical reactions or decompositions set in, in the viscose, which alter its physical and chemical properties and condition it for spinning and setting into a silk-like fiber. After the viscose has been properly ripened

or conditioned, it is spun by extruding or squirming it under pressure through the orifices of specially designed and constructed spinnerets, and is set as a continuous strand or filament in a precipitating or setting bath, which usually contains niter cake (NaHSO<sub>4</sub>), salt cake (Na<sub>2</sub>SO<sub>4</sub>), and free sulphuric acid. The wet precipitated filament may be wound on a spool or equivalent winding device, from which it may be unwound for subsequent treatment, such as washing, bleaching, twisting, or other operations carried out in connection with or incident to the preparation of thread.

The physical characteristics of the finished silk-like or artificial silk filament or thread thus produced are in great measure undoubtedly dependent upon the characteristics of the original cellulosic fiber employed as the raw material. For example, it is impossible to manufacture artificial silk of substantial or workable strength from ground wood, cheap soda pulp, or the usual unbleached kraft pulp. Even the ordinary unbleached sulphite pulp is unsuitable for such manufacture, and results in an inferior product which may be commercially worthless. While certain high grades of bleached sulphite pulp may be employed in the manufacture of artificial silk, the resulting product is usually inferior to one resulting from the employment of cotton linters as the raw cellulosic fibrous material; in other words, the strength and other desirable physical qualities in an artificial silk product are doubtless dependent upon the strength and alpha cellulose content of the cellulosic fibers or raw material from which it is prepared.

The purified or high alpha cellulose pulp prepared and utilized in the practice of the present invention for the preparation of the viscose may or may not possess papermaking characteristics, depending upon the strength of the caustic soda solution employed and the various conditions under which the purification treatment is effected, in contradistinction to the special conditions under which the purification reaction must be carried out where a substantially unmercerized high alpha cellulose fiber suitable as a rag substitute in papermaking is desired.

In my applications, Serial No. 26,361, filed April 28, 1925, and Serial No. 52,232, filed August 24, 1925, there are described meth-

ods for purifying pulp, and more especially sulphite pulp, for the production of a high alpha cellulose product especially suitable for conversion into cellulose derivatives. The 5 method described in the first mentioned application consists in treating unbleached sulphite pulp at an elevated temperature with a relatively dilute solution of caustic soda for a sufficient period of time to eliminate the 10 ligneous and less-resistant celluloses contained therein, resulting in a product high in resistant or alpha cellulose. The purified product may be bleached to high whiteness without the necessity of an excessive amount 15 of bleach and without affecting the strength or alpha cellulose content thereof, or otherwise injuring it appreciably.

The method described in the last mentioned application consists in treating pulp, 20 and more especially unbleached sulphite pulp, at ordinary or room temperature, with a relatively concentrated solution of caustic soda containing sufficient alkali to react with and remove less-resistant celluloses 25 contained in the pulp, but insufficient to cause a substantial mercerization of the alpha cellulose content thereof, thereby yielding a product notably high in alpha cellulose. The product thus obtained is easily 30 bleachable to high whiteness with a moderate amount of bleach, without substantially affecting its other properties.

It is thus to be observed that the same 35 reagent, viz, caustic soda, may be employed in purifying the unbleached pulp to produce a high alpha cellulose fiber especially suitable for conversion into a cellulose derivative such as viscose, and for converting the alpha cellulose into the soda cellulose, which constitutes the initial step of the viscose process.

Ordinarily a portion of the caustic soda liquor expressed from the pulp sheets in forming the soda cellulose is later converted into a sulphate solution which is employed in the setting bath. Such practice is followed because the liquor expressed from the sheet contains certain organic impurities dissolved from the pulp, and the re-use 50 of all such liquor for converting other sheets of pulp to soda cellulose would cause the impurities to become more highly concentrated, although the solution may be re-used, after the addition thereto of sufficient caustic soda to convert such other pulp into soda cellulose and to make up losses in caustic soda resulting from its previous use; however, the continued re-use of and treatment with such a solution would ultimately 55 not permit the purification incident to such treatment by the use of a fresh solution of caustic soda, since a condition of dynamic equilibrium is reached when the pressed sheets contain the amount of impurities contained therein before such treatment. Hence

a substantially fresh caustic soda solution is preferably employed in treating the pulp sheets for conversion into soda cellulose.

In accordance with the present invention, where the preparation of the viscose occurs 70 simultaneously or in connection with the preparation of a high alpha cellulose product for use in making such viscose, the caustic soda solution expressed from the sheets of pulp may be advantageously employed in 75 purifying other pulp to produce the high alpha cellulose fiber either by a hot or cold treatment, and the purified pulp is treated with a substantially fresh solution of caustic soda.

With the foregoing and other features in view, a more complete understanding of the present invention may be gained from the following description thereof when considered in conjunction with the accompanying 85 drawings, which may be termed a "flow sheet", and which shows the sequence of treatments and the progress of flow of the various materials.

Referring to the drawings, at 1, I have 90 indicated a storage tank containing a supply of pulp, preferably an unbleached sulphite pulp produced by the liberation of fiber under the proper conditions from wood chips (e. g., spruce) in a suitable acid sulphite liquor, and which is to undergo a purifying or refining treatment with a caustic soda solution preparatory to its conversion 95 into artificial silk by the viscose process. The pulp is delivered to a set of pulp thickeners 2, wherein the pulp is thickened to the desired consistency. The thickened pulp is then mixed with a sufficient amount of caustic soda liquor expressed from the sheets of previously purified or alpha pulp 100 in the pressing operation. The liquor expressed from the purified sheets in the viscose process is thus utilized to effect initial treatment or purification of the unbleached pulp. The pulp together with the solution 105 of caustic soda admixed therewith is delivered to a reaction tank 3 communicating at its lower portion by a slow-moving worm with a second reaction tank 4.

Where the pulp is to be purified by a cold 115 treatment, the stock undergoing purification in the tanks is preferably maintained at a stock consistency of about 5% to 6%, the treating liquor containing about 100% to 150% caustic soda based on the dry weight 120 of fiber. By regulating the degree of thickening and the amount of expressed liquor admixed therewith, such stock and caustic soda concentration may be produced. The purifying treatment is carried out preferably 125 while stirring or agitating the pulp so as to promote a uniform reaction at room temperature (say, 30° C.), and the purification reaction may require 30 minutes to two hours, depending on the characteristics of 130

the stock undergoing treatment. If desired, provision may be made to heat the stock undergoing treatment by introducing a certain amount of steam directly thereto, to maintain it within certain definite temperatures, preferably between 15° C. and 50° C., during seasons of the year when the water available is at too low a temperature.

While I have described the purification of sulphite pulp in a cold, relatively concentrated solution of caustic soda, this was by the way of illustration only, and, if desired, the purification of the pulp may be effected at an elevated temperature in a relatively dilute solution containing about 5% to 6% of caustic soda.

The resulting purified product, in either case, usually contains from about 94% to 98% alpha cellulose, and may be washed substantially free from entrained reaction products and from alkali, in a counter-current washer 5. The spent liquor which leaves the counter-current washer and is delivered to a storage tank 6 not only contains a very high percentage of residual unconsumed caustic soda, but the various organic substances removed from the original pulp. The liquor will vary from a light brown to a dark brown color, depending upon the character of the original raw fiber stock. A large portion of such spent liquor may be re-employed, as indicated on the drawing, for admixture with and in the treatment or purification of other raw sulphite pulp, and a portion may be withdrawn and the chemicals contained therein may be recovered as in connection with the hot process described in the application previously referred to. The diverted or withdrawn portion of spent liquor, however, may be converted into salt cake, by treatment with sulphuric acid, if desired, and may be employed in the preparation of the setting bath.

The washed alpha cellulose fiber is preferably bleached before conversion into viscose. To this end, the purified stock is passed into a storage tank 7, from which it is withdrawn and supplied to a set of thickeners 8, wherein it is concentrated to the consistency desired for bleaching. The concentrated stock from the thickeners is diluted to the desired consistency, say about 10% to 16%, with the required amount of bleach liquor delivered from a supply tank 9, and is passed into bleaching tanks 10 and 11, arranged in series, wherein the stock is bleached while agitated and at the required temperature for the necessary period of time. The amount of bleach required in the bleaching operation depends upon the characteristics of the initial raw pulp stock and the degree of purification effected by the alkaline treatment with caustic soda. Under ordinary conditions, about 5% to 8% of bleach, based on the weight of dry fiber, is required

to bring the stock up to the desired degree of whiteness. The stock after bleaching is delivered to a multiple washing machine 12, preferably of the Wolf type, and is washed substantially free of bleach solution 70 and entrained soluble reaction products prior to sheeting and conversion into soda cellulose.

The bleached, purified pulp, containing a high percentage of alpha cellulose, is passed 75 into a storage tank 13, from which it is supplied to a wet or cylinder machine 14 and formed into sheets and dried to a water content of about 10%. The sheets of purified pulp which are now prepared for conversion 80 into soda cellulose are delivered to a soaking bath 15, wherein they are immersed in a solution containing 16% to 20% caustic soda, until they are completely saturated therewith. The soaked sheets are then forwarded 85 to a suitable press 16, by means of which the excess caustic soda liquor is expressed therefrom, but sufficient caustic soda is left behind within the sheets for their conversion into soda cellulose. The sheets are then 90 aged under proper conditions in a storeroom 17, until the cellulose has undergone the necessary chemical change and has been converted into a soda cellulose, whereupon the soda cellulose thus formed is subjected to 95 the other treatments previously alluded to as being necessary for the manufacture of finished artificial silk filament.

The new caustic soda which is necessary for replacing sodium losses in the entire 100 purification cycle, as well as the sodium constituent accompanying the pressed sheets of purified pulp for the viscose process, is added to the soaking vat 15, provision being made to add sufficient caustic soda to the vat 105 15 to maintain a liquor containing 16% to 20% caustic soda. The caustic soda is preferably added in the form of a strong solution to replace the corresponding volume of solution removed therefrom by the sheets of 110 purified pulp. Due to reaction between the caustic soda solution and the small quantity of less stable celluloses contained in the purified pulp, as well as to the adsorption of a certain amount of caustic soda from the 115 solution by the sheets, the caustic soda liquor expressed from the pulp and passed into the storage tank 18 contains only about 15% to 18% of active caustic soda. As previously indicated and shown on the drawing, this expressed liquor is utilized in accordance with the present invention for admixture with the raw pulp to be purified, as it is fairly free from contamination, and possesses sufficient unreacted or free caustic 120 soda to be used for the initial purification 125 of the raw pulp.

At times, all the press liquor available from the pressing operation may be necessary in the treatment of the raw pulp to be 130

purified. Under certain conditions of operation, however, it may occur that there is more press liquor available than necessary for effecting the purification of the raw or unrefined pulp. This may especially be the case where a hot treatment with a dilute solution of caustic soda is employed for effecting such purification. In such cases, the excess portion of the press liquor which is not needed in the purification treatment may be returned to the soaking vat, as indicated, in which case the volume of caustic soda solution supplied thereto at a somewhat higher concentration will correspond substantially to the volume removed therefrom by the sheeted purified pulp minus that portion which is returned or re-employed from the pressing operation; or the excess portion may be diverted for use in the setting bath after conversion into salt cake; or a procedure may be followed wherein a fraction of the excess press liquor is employed for the preparation of the setting bath and the remaining fraction is re-employed in the soaking vat.

By the practice of the hereinbefore described process, it is obvious that one may employ that portion of the press liquor for the purification of the initial raw pulp, which is ordinarily later converted into sodium sulphate. Thus the losses encountered in the purification cycle are made up by the addition of a fresh caustic soda solution to the soaking vat, so that a substantially fresh solution of caustic soda is maintained practically at all times for the soaking of the purified sheets of pulp, and the production of a high grade artificial silk product or filament is ensured. Such an artificial silk is of notably high strength as compared to the artificial silk product obtainable from the usual untreated pulps by the viscose process, and hence compares more favorably with a product made from cotton linters.

While I have confined the description of the process of this invention as exemplified by the use of unbleached sulphite pulp as the raw material, it is equally applicable in processes wherein other pulps such as kraft or certain grades of soda pulp are first subjected to a purification treatment with caustic soda, and the pulp thus treated is subsequently converted into cellulose xanthate or viscose, as herein described.

Before concluding, it may be stated that by employing a purification treatment of raw pulp wherein a relatively concentrated solution of caustic soda is employed at low temperature, a somewhat larger alpha cellulose content, and a smaller yield, which is reduced relatively to a greater extent than the increase in alpha cellulose, is obtained than when such pulp is purified with a relatively dilute solution of caustic soda at an

elevated temperature. The characteristics of the purified or high alpha cellulose pulp depend upon the type of treatment employed, the cold treatment with a relatively concentrated solution of caustic soda yielding a purified pulp which is notably low in pentosan content and which is generally more suitable for conversion into cellulose xanthate. However, where the pentosan content is immaterial in certain grades of viscose, the hot treatment with a relatively dilute solution of caustic soda may be employed.

Having thus described this invention, it should be obvious that various changes and modifications might be resorted to in the procedure without departing from the spirit or scope of invention as defined by the appended claims.

What I claim is:

1. An interrelated pulp-purifying and viscose process which comprises the following steps, to-wit: treating pulp with a solution containing caustic soda, to effect the purification thereof; washing the purified pulp; sheeting said pulp; soaking the sheeted material with a solution of caustic soda preparatory to conversion into viscose; expressing the excess caustic soda solution from said sheets; and employing such expressed liquor in said first mentioned step for the like treatment of other pulp.

2. A cyclic process of treating pulp in the production of viscose, which comprises soaking purified pulp in a bath comprising a solution of caustic soda, removing the pulp therefrom and expressing excess caustic soda solution therefrom; and purifying raw pulp for such soaking treatment by said expressed caustic soda solution.

3. A cyclic process of treating pulp in the production of viscose, which comprises continuously feeding a stream of pulp through and soaking it in a bath of caustic soda solution, expressing excess solution therefrom, continuously supplying the expressed solution to the stream of pulp prior to its being fed to the soaking bath to purify such pulp, continuously washing such stream of pulp after reaction with such expressed solution and prior to its being fed to the aforesaid bath, and supplying fresh caustic soda solution to said bath to make up losses therein.

4. In the manufacture of viscose, a process which comprises feeding a mass of pulp, previously purified by treatment with a solution containing caustic soda, to and soaking it in a bath of caustic soda solution preparatory to its conversion into viscose; continuously expressing the excess caustic soda solution from said mass but allowing sufficient caustic soda to remain therein for its conversion into soda cellulose; supplying a portion of the expressed excess solution to a mass of pulp for the purification thereof

prior to its being fed to such bath, and returning a portion of such expressed solution to said bath.

5. A process which comprises soaking a mass of pulp, previously purified by treatment with a solution containing caustic soda, in a bath of caustic soda solution preparatory to its conversion into viscose; removing said mass from said bath and expressing 10 the excess caustic soda solution from said mass but allowing sufficient caustic soda to remain therein for its conversion into soda cellulose; treating raw pulp with such expressed solution for the purification thereof 15 prior to its being soaked in said bath; and adding caustic soda to said bath sufficient to make up sodium losses therein due to the purification of such pulp and to the removal therefrom of a portion of the caustic soda 20 necessary for the conversion of said pulp to soda cellulose.

6. An interrelated pulp-purifying and viscose process which comprises the following steps, to wit: feeding a stream of raw 25 pulp and a solution containing caustic soda through a reaction chamber to effect the purification of such pulp; washing the purified pulp delivered therefrom; sheeting said pulp; soaking the sheeted material in a 30 bath of caustic soda preparatory to conversion into viscose; removing the sheets from the bath and expressing the excess caustic soda solution therefrom, and circulating such expressed solution back to the 35 reaction chamber for the purification of the stream of raw pulp.

7. An interrelated pulp-purifying and viscose process which comprises the following steps, to wit: digesting raw pulp in a 40 bath of caustic soda solution to effect the purification of such pulp; washing the purified pulp; sheeting said pulp; soaking the sheeted material in a bath of caustic soda solution preparatory to its conversion into 45 viscose; removing the sheets from the bath and expressing the excess caustic soda solution therefrom; and circulating a portion of such expressed solution to said first mentioned purifying bath and circulating the 50 remaining portion to the soaking bath.

8. An interrelated pulp-purifying and viscose process which comprises digesting raw pulp in a bath of caustic soda solution to effect a purification of such pulp; washing 55 the purified pulp; sheeting such pulp; soaking such sheeted material in a solution of caustic soda preparatory to its conversion into viscose; removing the sheets from the bath and expressing the excess caustic 60 soda solution from said sheets, but allowing sufficient caustic soda to remain therein for its conversion into soda cellulose; circulating such expressed solution to said first men-

tioned purifying bath, and adding sufficient caustic soda to said soaking bath to make up 65 sodium losses incident to the purification of such pulp and to the removal therefrom of a portion of the caustic soda necessary for the conversion of said pulp to soda cellulose.

9. An interrelated pulp-purifying and viscose process which comprises digesting raw pulp in a bath of caustic soda solution to effect a purification of such pulp; separating the purified pulp from the solution; reemploying the solution for the digestion 70 of other pulp; sheeting the purified pulp; soaking such sheeted material in a bath of caustic soda solution preparatory to xanthation; removing the sheets from the bath and expressing the excess caustic soda solution from said sheets; circulating such expressed solution to said first-mentioned purifying bath; and adding sufficient caustic soda to 75 said soaking bath to make up sodium losses incident to the purification of such pulp and to the removal therefrom of a portion of the caustic soda necessary for xanthation. 80

10. An interrelated pulp-purifying and viscose process which comprises digesting raw pulp in a bath of caustic soda solution to effect a purification of such pulp; separating the purified pulp from the solution; re-employing a portion of the solution for digestion of other pulp and employing a portion 90 for the viscose setting bath; sheeting the purified pulp; soaking such sheeted material in a bath of caustic soda solution preparatory to its xanthation, removing the sheets from the bath and expressing the excess caustic soda solution from said sheets; circulating such expressed liquor to said first mentioned purifying bath; and adding sufficient caustic soda to said soaking bath to 95 make up sodium losses incident to the purification of such pulp and to the removal therefrom of a portion of the caustic soda necessary for xanthation. 100

11. An interrelated pulp-purifying and viscose process which comprises digesting raw pulp in a bath of caustic soda solution to effect a purification of such pulp; separating the purified pulp from the solution; re-employing the solution for the digestion 110 of other pulp; bleaching the purified pulp and washing the bleached product; sheeting the bleached and washed pulp; soaking said sheets in a bath of caustic soda solution preparatory to its xanthation; removing the sheets from the bath and expressing the excess caustic soda liquor from said sheets, and circulating such expressed solution to 115 said first-mentioned purifying bath. 120

In testimony whereof I have affixed my signature.

GEORGE A. RICHTER.